

Dec. 1, 1925.

1,564,185

C. B. SEEM

METHOD OF CASTING RADIATOR SECTIONS AND THE LIKE

Original Filed Oct. 7, 1924

FIG. 2.



FIG. 1.



FIG. 3.



FIG. 4.



*Herman Jakobson*

By

Attorney



Patented Dec. 1, 1925.

1,564,185

# UNITED STATES PATENT OFFICE.

CHARLES B. SEEM, OF WILLIAMSPORT, PENNSYLVANIA.

## METHOD OF CASTING RADIATOR SECTIONS AND THE LIKE.

Original application filed October 7, 1924, Serial No. 742,141. Divided and this application filed April 27, 1925. Serial No. 26,209.

To all whom it may concern:

Be it known that I, CHARLES B. SEEM, a citizen of the United States, residing at Williamsport, in the county of Lycoming and 5 State of Pennsylvania, have invented certain new and useful Improvements in Methods of Casting Radiator Sections and the like, of which the following is a specification.

10 The present invention relates to an improved method of casting radiator sections and the like using permanent molds for carrying out the same, this being a divisional application of my copending application 15 for "permanent molds", Ser. No. 742,141, filed October 7, 1924.

The usual method of producing radiator section castings is to provide individual molds built up in sand for each casting 20 which is a very costly and tedious procedure.

The introduction of my molds and process for doing the work in radiator plants and other duplicating foundries, independent of 25 what kind of metals or alloys are employed, means a considerable saving in time and labor, and a consequent reduction in prices of the articles so produced.

In carrying out my invention I make use 30 of a two-piece metal mold, having a collapsible core, such as baked sand suspended in a fixed position in the hollow part of the mold between the cope and the drag.

The mold employed for carrying out this 35 process is illustrated in the accompanying drawing in which—

Fig. 1 represents a top plan view of the mold;

Fig. 2 an end view of Fig. 1, partly in 40 section with the mold closed;

Fig. 3 a longitudinal section along line 3—3 of Fig. 1 with the core and casting in position;

Fig. 4 a plan view of the mold open exposing the recesses and channels for the casting; and

Fig. 5 a cross section along line 5—5 of Fig. 1.

In the drawing, reference numeral 10 50 represents the cope or top half of the mold, and reference numeral 11 the drag or bottom part thereof. For radiator sections both halves are identical and have been shown such in the drawing, but it is evident 55 that the cope and the drag may have entirely different cavities depending on the

section and contour of the casting for which the mold is intended. The mold is to be properly vented and is preferably of rectangular form, the two halves being hinged 60 together along one side as at 12 and provided with clips or clamps 13 on the other side. The hollow portion of the mold consists of recesses 14 in each half for the body of the radiator section and channels 15 for 65 the radiating fins thereon. Shallow depressions 16 may also be provided to form bridges between the walls of the casting and at each end is furnished a pocket 17 for forming the contacting pads 25 between the 70 sections. In order to properly position the core in length direction of the mold these pockets 17 may have a smaller concentric depression as at 18.

Sufficient metal is provided outside the 75 main recess 14 along all edges of the mold so that the surfaces 19 at the central dividing plane of the mold make proper contact to prevent leakage. At 20 is shown the gate, one half on each side of the dividing 80 plane. From this gate leads 21 radiate and open into the main recess 14.

The core 22 is collapsible and consists 85 preferably of hard packed sand into which are baked short metal pins or chaplets 23 which are of a length corresponding to the height of the cavity of the mold so that the ends of the chaplets abut against the top and bottom of the cavity. In this manner the core becomes freely suspended in the 90 cavity so that walls 26 of even thickness are obtained in the casting. As already described the core may be positioned accurately in length direction by engaging with suitable lugs 24 in the depressions 18. 95

The interior surfaces of the mold such as the recesses 14, channels 15 and pockets 17 are carbonized by a torch in order to form a film and prevent the poured metal from freezing to the mold. 100

Before commencing the casting operation the mold preferably containing the core is heated to a sufficient degree to prevent chilling the casting. The pouring of the metal is then started by the aid of either 105 pneumatic pressure, vacuum or gravity.

As soon as the casting has been completed and the metal has become solid the locking clamps 13 are removed and the cope 10 110 swung open or raised, thus exposing the casting which then may be lifted out of the drag 11. The core 22 is next taken out

through the end openings at 18 and the interior of the casting cleaned in the usual manner. The pins or supporting inserts 23 will then remain in the casting and form 5 supports for the walls.

Some of the advantages gained by the use of this casting method are: practically perfect castings and no chipping or dressing necessary as the chaplets are permitted to 10 remain in the casting supporting the walls.

What I claim as new is:

A method of producing metal castings

consisting in first carbonizing the cavities of a metal mold; second placing inserts in the core of the mold adapted to hold the 15 core in position but primarily to act as supporting braces for the cast walls; third heating the mold to prevent chilling; fourth pouring metal into the mold and lastly removing the core from the casting when solid 20 permitting the inserts to remain in the casting.

In testimony whereof I affix my signature.

CHARLES B. SEEM.